

April 25, 1961

E. ALBERS-SCHOENBERG

2,981,688

FERRITES FOR MICROWAVE APPLICATIONS

Filed May 27, 1960



INVENTOR.  
ERNST ALBERS-SCHOENBERG

BY  
Greene, Pineles & Durr

ATTORNEYS

# United States Patent Office

2,981,688

Patented Apr. 25, 1961

1

2

2,981,688

## FERRITES FOR MICROWAVE APPLICATIONS

Ernst Albers-Schoenberg, Redfield Village, Metuchen, N.J., assignor, by mesne assignments, to Steatite Research Corporation, Keasbey, N.J., a corporation of Delaware

Filed May 27, 1960, Ser. No. 32,387

5 Claims. (Cl. 252—62.5)

This application relates to devices known as ferrite gyrator elements or ferrite direction inverters and to Faraday plates which are an essential part of the former.

This application is a continuation-in-part of U.S. application Serial No. 352,205, filed April 30, 1954, now abandoned, which application in turn is a continuation-part of U.S. application Serial No. 67,752, filed December 28, 1948, also abandoned. In application Serial No. 67,752 an unusual type of ferrite material is disclosed. Whereas the ordinary ferrite has a formula of

$$xM\text{O}_y\text{Fe}_2\text{O}_3$$

in which M represents one or more bivalent metal oxides and in which  $x:y$  is approximately 1:1, the ferrites disclosed in said application Serial No. 67,752 have an  $x:y$  ratio which is between 1.2:1 and 3:1 and preferably between 1.6:1 and 2:1. These ferrites utilize MgO as the essential bivalent oxide.

Application Serial No. 352,205 discloses that a certain group of ferrites disclosed in U.S. application Serial No. 67,752 having an  $x:y$  ratio of 1.2:1 to 3:1, have unusual properties making them particularly suitable as Faraday plates in ferrite gyrator elements.

One objection to the ordinary ferrite gyrator elements relates to their high losses. It is among the objects of this invention to provide a Faraday plate for a ferrite gyrator element which has very low losses in such applications.

Among other objects of the invention is to provide a ferromagnetic ferrite having low dielectric losses especially useful for microwave applications.

Another object of the invention is to provide a new and improved ferrite gyrator element.

The foregoing objects and other objects of the invention will be best understood from the following description of exemplifications of the same when read in connection with the accompanying drawing in which the single figure is a perspective view partly in cross section of a circuit element embodying the features of the invention.

Recently, the gyrator elements, referred to above, comprising wave guides including ferrite cores, have evolved as new circuit elements for microwave frequencies. Such gyrator elements are useful for phase changers, modulators and switches, for example.

This type of new circuit element is a unique device, since it violates the law of reciprocity; that is, it does not have similar properties in both directions equally. The plane of polarization of microwave propagation can be changed as the wave passes through the ferrite which is magnetized with a steady field. This device can properly be called a ferrite gyrator element. The ferrite core has been named a Faraday plate. The actual effect upon electromagnetic microwave radiation is similar to the Faraday rotation of the plane of polarization in optics where a steady or static magnetic field is parallel to the direction of propagation through a transparent isotropic medium.

In general terms the rotation effect is due to the interaction of:

(1) The spinning electrons which will precess about a force not parallel to their axis of spin (similar to a gyroscope),

(2) A steady magnetic field parallel to the direction of propagation which acts as the aligning force on the gyroscopic spinning electrons in the ferrite,

(3) Circularly polarized waves in the wave guide which are propagated through the ferrite.

Actually, circularly polarized waves are not necessary since any linearly polarized wave can be considered as the resultant of two circularly polarized components of equal amplitudes which are rotating in opposite directions with equal angular velocities. Thus, one direction of circular polarization will be in the same direction as the precession of the elemental electron gyroscope and the other direction of circular polarization will be in the opposite direction to that of the precession. It is evident that one component of circular polarization which has the same sense of circular direction as the precession of the elemental electron gyroscope in the ferrite will be rotated more than the normal amount due to angular velocities, while the other circularly polarized wave of the opposite direction will be rotated only the normal amount, or less than that, due to its angular velocity. Thus, at the exit end of the ferrite, there will be a relative phase shift between both circularly polarized components. When these are combined again into the linearly polarized wave, the plane of polarization of the latter is shifted with respect to the plane of polarization before it entered the ferrite. Another way of looking at this phenomenon is to consider it as a relative change of the velocities of propagation of the circularly polarized waves.

If very much attenuation of both circularly polarized waves occurs due to the loss characteristic of the ferrite, then its efficiency as a transparent medium is poor. If the two circularly polarized waves which emerge from the ferrite are attenuated unequally, then an elliptically polarized wave will result.

Different ferrites vary as to their attenuation properties (or loss characteristics), ellipticity (or unequal attenuation of the two circularly polarized waves), and rotation. In addition, as one would expect, these properties vary as a function of the steady magnetic field. Also, there is a resonance point present when the precession frequency of the elemental electron gyroscopes coincides with that of the microwave frequency. This point is characterized by complete absorption of the interacting circularly polarized wave, and thus, very high losses.

Losses in a Faraday plate or ferrite cores of such devices may comprise dielectric losses, magnetic losses or may be due to some other unknown quality of the core. For example, it is believed that the low losses and effectiveness of the core of the present invention are not only due to its magnetic and dielectric properties but that they are, in some way, associated with the presence of more than one crystalline phase in the material due to the low proportion of  $\text{Fe}_2\text{O}_3$  with respect to the bivalent metal oxides.

The ferrites employed in the gyrator of this invention not only have low losses but combine with this property a fairly high rotation. These two properties are both desirable in a Faraday plate.

The ferrites of the gyrator element of this invention comprise compositions which are essentially of the formula  $x(\text{MgO}, \text{MO})_y\text{Fe}_2\text{O}_3$  in which the MO represents a heavy metal oxide which is less than 10% by weight of the entire composition (with the exception of MnO which may be added in amounts up to 20% of the composition) and in which  $x:y$  is between 1.2:1 and 3:1.

The MO may be entirely absent and may be MnO, ZnO, CdO, CuO, NiO or any similar bivalent oxide. When added the said MO acts as a flux to reduce the maturing temperature below what it is for the substantially pure  $x\text{MgO}, y\text{Fe}_2\text{O}_3$ . To be effective as a flux the MO should be present in amounts of from 1-20% of the total weight of the product. As indicated the MnO is especially desirable in that in addition to acting as a flux, it may improve the desirable properties of the  $\text{MgOFe}_2\text{O}_3$ . The MnO may be added in addition to the other bivalent oxide fluxes until a total of 20% of flux is obtained although with no more than 10% of the other bivalent oxide fluxes.

Ferrites within the limits specified but containing over 55 mol percent of MgO are very satisfactory since they have a low susceptibility to compositional variations and may therefore be made with very uniform properties. Increasing the MgO content to 55 mol percent reduces the maximum allowable iron oxide content to 44 mol percent and the maximum amount of MnO to 22 mol percent.

The properties of such ferromagnetic bodies which probably relate to their application in gyrator elements are as follows:

- (a) Initial permeability ( $\mu_0$ ) 10-40 at 1 mc.
- (b) Saturation magnetization,  $B_s$ , of approximately 1500 gaussess.
- (c) Dielectric constant of about 8 to 20.
- (d) Low magnetic losses at 1 mc.
- (e) Relatively low dielectric losses,  $\tan \delta$ , of about .05 at 1 mc. and about .001 at  $10^{10}$  c.p.s.

The dielectric constant of such bodies does not substantially change up to 10,000 mcs. However, the dielectric constant at these frequencies is difficult to measure with accuracy. The initial permeability at 10,000 mcs. may be as low as unity. The magnetic losses at 10,000 mcs. vary somewhat, but are, at least, by one order of magnitude smaller than that of other ordinary ferrite materials.

The device shown in the drawing has a first rectangular wave guide 10 and a second rectangular wave guide 11 connected by a circular tube 12 in which the Faraday plate or ferrite 20 is placed. A magnetizing coil 21 surrounds the central portion of the circular tube 12 to magnetize the ferrite plate 20. Depending on the thickness of the plate or length of the ferrite 20, the amount of magnetization, etc., the wave in guide 11 will be rotated a certain number of degrees, in a clockwise direction,  $90^\circ$ , for example. If any wave of the same frequency, etc., is passed from guide 11 through plate 20 and then to guide 10 this wave will be rotated  $90^\circ$  by plate 20 but if passed in a counter direction will not be rotated in the opposite direction (as would be expected by the law of reciprocity) but in the same direction. Any reflected wave would therefore be  $180^\circ$  out of phase with respect to the original wave. In the device shown, the central circular tube 12 is about the diameter of an ordinary cigarette.

#### EXAMPLE 1

A ferrite core is made by grinding, mixing and firing a composition of the following ingredients in the proportions disclosed:

|                                        | Parts by weight |
|----------------------------------------|-----------------|
| Calcined magnesite                     | 21              |
| Magnesium fluoride                     | 1               |
| Manganese dioxide                      | 6               |
| Zinc oxide                             | 1               |
| Iron oxide ( $\text{Fe}_2\text{O}_3$ ) | 71              |

This provides a product with the following molar ratio 1.24 ( $\text{MgO}:\text{MgF}_2$ ), 0.16 MnO, 0.03 ZnO:1  $\text{Fe}_2\text{O}_3$  the ratio of  $x:y$  being approximately 1.43:1.

This product can be fired at  $1360^\circ \text{C}$ . due to the presence of ZnO,  $\text{MgF}_2$  and MnO which act as fluxes.

The product has the following properties:

|                             |                         |
|-----------------------------|-------------------------|
| Specific resistance         | $0.8 \times 10^9$ ohms. |
| Power factor, $\tan \delta$ | $170 \times 10^{-4}$ .  |
| Initial permeability        | (Approx.) 30.           |
| Dielectric constant         | About 10.               |

At 10,000 mcs. the initial permeability is about 1.0.

#### EXAMPLE 2

A ferrite core is made of the following composition

|                            | Parts by weight           |
|----------------------------|---------------------------|
| Magnesium oxide            | 25                        |
| Magnesium fluoride         | 3                         |
| Manganese dioxide          | 6                         |
| Iron oxide                 | 66                        |
| Approximate ratio of $x:y$ | = 1.8:1.                  |
| Firing temperature         | = $1390^\circ \text{C}$ . |

This body has lower magnetic losses at 10,000 mcs. than the body of Example 1 and represents an improvement over such body in this respect.

When these bodies are inserted in the device of the drawing as the plate 20 in diameter of .6 cm. f.e. a gyrator element having exceptionally low losses and good performance is produced. The measurements of rotation were obtained on samples of 1 inch or 2.54 cm. length. Such circuit elements are useful for one-way transmitting devices, for example, and since the rotation of the wave may be controlled by an external source of the magnetizing current they may also be used in electrically controlled attenuators, modulators and microwave switches.

The following tables give the essential features of further examples.

#### EXAMPLES 3-6

|    |                                       | Example 3      | Example 4     | Example 5      | Example 6        |
|----|---------------------------------------|----------------|---------------|----------------|------------------|
|    |                                       | Mol. Per. cent | Wt. Per. cent | Mol. Per. cent | Wt. Per. cent    |
| 40 | MgO                                   | 58             | 24.3          | 58             | 28.1             |
|    | MnO                                   | 2              | 1.9+          | 10             | 10.5             |
|    | NiO                                   |                |               | 14             | 18.2             |
|    | Fe <sub>2</sub> O <sub>3</sub>        | 40             | 71.8          | 32             | 61.5             |
| 45 | Rotation, 2.54 cm. or 1 inch, degrees | 202            | Low           | 176            | Low              |
|    | Losses                                |                |               | 162            | Low              |
|    |                                       |                |               |                | 212              |
|    |                                       |                |               |                | Low <sup>1</sup> |

<sup>1</sup> But slightly higher than for Examples 3-5.

#### EXAMPLES 7-11

|    | Ex. 7, Wt. Per. cent                            | Ex. 8, Wt. Per. cent | Ex. 9, Wt. Per. cent | Ex. 10, Wt. Per. cent | Ex. 11, Wt. Per. cent |
|----|-------------------------------------------------|----------------------|----------------------|-----------------------|-----------------------|
| 55 | MgO                                             | 25                   |                      | 30                    |                       |
|    | MgCO <sub>3</sub>                               |                      | 44                   |                       | 48                    |
|    | MgF <sub>2</sub>                                | 3                    |                      | 3                     |                       |
|    | MnO                                             | 8                    |                      | 6                     |                       |
|    | Mn <sub>2</sub> O <sub>3</sub> H <sub>2</sub> O |                      | 4.5                  |                       | 4.5                   |
|    | Fe <sub>2</sub> O <sub>3</sub>                  | 66                   | 51.5                 | 61                    | 47.5                  |
| 60 | Mol ratio                                       | 1.8                  | 1.8                  | 2.3                   | 2.3                   |
|    | <u>MgO+MO</u>                                   |                      |                      |                       |                       |
|    | <u>Fe<sub>2</sub>O<sub>3</sub></u>              |                      |                      |                       |                       |

Examples 7 and 8 produce substantially the identical composition after firing and similarly Examples 9 and 10 produce the same end product. Example 11 illustrates a body prepared without additional flux. In order to obtain a satisfactory product from this composition the materials are mixed, fired at around  $1400^\circ \text{C}$ . and thereafter refined several times.

Examples 7 and 8 have low losses and a rotation of approximately  $220^\circ$  per inch.

Examples 9 and 10 have low losses and a rotation of approximately  $180^\circ$  per inch.

Example 11 has low losses and a rotation of approximately  $80^\circ$  per inch.

When the term "low losses" is employed it means that the losses are below 1.0 decibel, for example.

The features and principles underlying the invention described above in connection with specific exemplifications will suggest to those skilled in the art many other modifications thereof. It is accordingly desired that the appended claims shall not be limited to any specific features and details shown and described in connection with the exemplifications thereof.

I claim:

1. A ferromagnetic ferrite consisting essentially of a composition of the general formula



in which MO consists of at least one bivalent metal oxide selected from the group consisting of  $\text{ZnO}$ ,  $\text{CuO}$  and  $\text{NiO}$ , in which  $x:y$  is between 1.2:1 and 3:1, the total amount of MO being less than 10% by weight of the entire composition, the amount of  $\text{MnO}$  being at least 1% and no more than 20% by weight of said composition, and the total amount of MO and  $\text{MnO}$  being no more than 20% by weight of said composition, said ferrite having low dielectric losses,  $\tan \delta$ , of no more than about 0.05 at 1 mc. and of no more than about 0.001 at  $10^{10}$  c.p.s.

2. The ferrite of claim 1 in which the ratio of  $x:y$  is between 1.6:1 and 3:1.

3. A ferromagnetic ferrite consisting essentially of a composition of the general formula  $x(\text{MgO}, \text{MnO})_y\text{Fe}_2\text{O}_3$  in which  $x:y$  is between 1.2:1 and 3:1, the total amount of manganese oxide being between 1 and 20% by weight

of the entire composition, said ferrite having low dielectric losses,  $\tan \delta$ , of no more than about 0.05 at 1 mc. and of no more than about 0.001 at  $10^{10}$  c.p.s.

4. In a ferrite gyrator, a Faraday plate consisting essentially of a ferromagnetic plate of the composition of claim 3.

5. A fired, shaped ferrite body having low dielectric losses,  $\tan \delta$ , of no more than about 0.05 at 1 mc. and of no more than about 0.001 at  $10^{10}$  c.p.s., formed by firing at a temperature of about  $1390^\circ \text{C}$ , about 25 parts by weight of  $\text{MgO}$ , about 3 parts by weight of magnesium fluoride, about 6 parts by weight of manganese oxide calculated as  $\text{MnO}_2$ , and about 66 parts by weight of ferric oxide.

15

References Cited in the file of this patent

UNITED STATES PATENTS

|           |                   |                |
|-----------|-------------------|----------------|
| 2,565,861 | Leverenz et al.   | Aug. 28, 1951  |
| 2,576,456 | Harvey            | Nov. 27, 1951  |
| 2,640,813 | Berge             | June 2, 1953   |
| 2,644,930 | Luhrs et al.      | July 7, 1953   |
| 2,715,109 | Albers-Schoenberg | Aug. 9, 1955   |
| 2,719,274 | Luhrs             | Sept. 27, 1955 |
| 2,745,069 | Hewitt            | May 8, 1956    |
| 2,748,353 | Hogan             | May 29, 1956   |
| 2,877,183 | Eckert            | Mar. 10, 1959  |
| 2,886,530 | Greger            | May 12, 1959   |

FOREIGN PATENTS

|         |               |                |
|---------|---------------|----------------|
| 697,219 | Great Britain | Sept. 16, 1953 |
| 735,375 | Great Britain | Aug. 17, 1955  |